



US011040250B2

(12) **United States Patent**  
**Kuntimaddi et al.**

(10) **Patent No.:** **US 11,040,250 B2**  
(45) **Date of Patent:** **Jun. 22, 2021**

(54) **COATINGS FOR GOLF BALLS HAVING A THERMOPLASTIC POLYURETHANE COVER**

(71) Applicant: **Acushnet Company**, Fairhaven, MA (US)

(72) Inventors: **Manjari Kuntimaddi**, Raynham, MA (US); **Scott Cooper**, East Freetown, MA (US); **Matthew F. Hogge**, Plymouth, MA (US)

(73) Assignee: **Acushnet Company**, Fairhaven, MA (US)

(\*) Notice: Subject to any disclaimer, the term of this patent is extended or adjusted under 35 U.S.C. 154(b) by 0 days.

(21) Appl. No.: **16/590,179**

(22) Filed: **Oct. 1, 2019**

(65) **Prior Publication Data**

US 2021/0093926 A1 Apr. 1, 2021

(51) **Int. Cl.**

*A63B 37/06* (2006.01)  
*A63B 37/00* (2006.01)

(52) **U.S. Cl.**

CPC ..... *A63B 37/0022* (2013.01); *A63B 37/0027* (2013.01); *A63B 37/0031* (2013.01); *A63B 37/0033* (2013.01); *A63B 37/0075* (2013.01)

(58) **Field of Classification Search**

CPC ..... A63B 45/00; A63B 37/0022  
USPC ..... 473/409, 378

See application file for complete search history.

(56)

**References Cited**

U.S. PATENT DOCUMENTS

|              |           |                    |
|--------------|-----------|--------------------|
| 5,000,458 A  | 3/1991    | Proudfoot          |
| 5,461,109 A  | * 10/1995 | Blair .....        |
|              |           | A63B 37/0003       |
|              |           | 473/378            |
| 5,820,491 A  | * 10/1998 | Hatch .....        |
|              |           | A63B 37/0003       |
|              |           | 473/378            |
| 5,840,788 A  | * 11/1998 | Lutz .....         |
|              |           | A63B 37/0003       |
|              |           | 524/95             |
| 6,117,024 A  | 9/2000    | Dewanjee           |
| 6,190,268 B1 | 2/2001    | Dewanjee           |
| 6,395,861 B1 | * 5/2002  | Kennedy, III ..... |
|              |           | A63B 37/12         |
|              |           | 528/80             |
| 6,476,176 B1 | 11/2002   | Wu                 |
| 6,528,578 B2 | 3/2003    | Wu                 |
| 6,685,579 B2 | 2/2004    | Sullivan           |
| 7,118,497 B2 | 10/2006   | Sullivan et al.    |
| 7,131,915 B2 | 11/2006   | Sullivan et al.    |
| 9,044,648 B2 | 6/2015    | Sullivan et al.    |
| 9,333,396 B2 | 5/2016    | Comeau et al.      |
| 9,962,577 B1 | * 5/2018  | Chavan .....       |
|              |           | A63B 37/0076       |

(Continued)

FOREIGN PATENT DOCUMENTS

WO 2014149204 9/2014

Primary Examiner — Raeann Gorden

(74) Attorney, Agent, or Firm — Mandi B. Milbank

(57) **ABSTRACT**

Methods for coatings for golf balls, particularly golf balls having thermoplastic polyurethane covers, and the resulting finished balls are provided. The coating is preferably a topcoat comprising a polyurethane composition containing optical brighteners. The topcoat composition may comprise a low concentration of optical brighteners. For example, the concentration of optical brightener can be in the range of 0.01 to about 0.20 weight %. Multi-piece golf balls having inner cores, outer cores, inner covers, and intermediate layers can be made. The finished ball with the topcoat has many advantageous physical and playing performance properties.

**3 Claims, 3 Drawing Sheets**



(56)

**References Cited**

U.S. PATENT DOCUMENTS

- 2004/0176184 A1\* 9/2004 Morgan ..... C08G 18/10  
473/371  
2006/0089419 A1\* 4/2006 Hogge ..... C09D 175/16  
522/174  
2014/0274473 A1\* 9/2014 Yontz ..... A63B 45/00  
473/378

\* cited by examiner



FIG. 1



FIG. 2



FIG. 3



FIG. 4



FIG. 5



FIG. 6

## 1

**COATINGS FOR GOLF BALLS HAVING A  
THERMOPLASTIC POLYURETHANE  
COVER**

BACKGROUND OF THE INVENTION

Field of the Invention

The present invention generally relates to coatings for golf balls, particularly golf balls having thermoplastic polyurethane covers. The coating is preferably a topcoat comprising a polyurethane composition containing optical brighteners. Multi-piece golf balls having inner cores, outer cores, inner covers, and intermediate layers can be made. The invention includes methods for applying the coatings to the thermoplastic polyurethane cover. The finished ball with the topcoat has many advantageous physical and playing performance properties.

Brief Review of the Related Art

Both professional and amateur golfer use multi-piece, solid golf balls today. Basically, a two-piece solid golf ball includes a solid inner core protected by an outer cover. The inner core is made of a natural or synthetic rubber such as polybutadiene, styrene butadiene, or polyisoprene. The cover surrounds the inner core and may be made of a variety of materials including ethylene acid copolymer ionomers, polyamides, polyesters, polyurethanes, and polyureas.

Three-piece, four-piece, and even five-piece balls have become more popular over the years. More golfers are playing with these multi-piece balls for several reasons including new manufacturing technologies, lower material costs, and desirable ball playing performance properties. Many golf balls used today have multi-layered cores comprising an inner core and at least one surrounding outer core layer. For example, the inner core may be made of a relatively soft and resilient material, while the outer core may be made of a harder and more rigid material. The "dual-core" sub-assembly is encapsulated by a single or multi-layered cover to provide a final ball assembly. Different materials are used in these golf ball constructions to impart specific properties and playing features to the ball.

For instance, ionomer compositions comprising an ethylene acid copolymer containing acid groups that are at least partially neutralized can be used to make golf ball covers. Suitable ethylene acid copolymers that may be used to form the cover layers are generally referred to as copolymers of ethylene;  $C_3$  to  $C_8$   $\alpha$ ,  $\beta$ -ethylenically unsaturated mono- or dicarboxylic acid; and optional softening monomer. Commercially available ionomer compositions that can be used to make such covers include Surlyn® (DuPont) and Escor® and Iotek® (Exxon) ionomers.

In recent years, there has been high interest in using polyurethane compositions to make golf ball covers. Basically, polyurethane compositions contain urethane linkages formed by reacting an isocyanate group ( $—N=C=O$ ) with a hydroxyl group ( $OH$ ). Polyurethanes are produced by the reaction of a multi-functional isocyanate with a polyol in the presence of a catalyst and other additives. The chain length of the polyurethane prepolymer is extended by reacting it with hydroxyl-terminated and amine curing agents.

Different molding operations can be used to form the cover over the core or sub-assembly of the ball. For example, compression-molding, casting, and injection-molding processes can be used. These molding processes normally use molds having an upper mold cavity and lower

## 2

mold cavity. Each mold cavity is hemispherical-shaped and one-half of the size of a finished ball. The mold cavities have interior walls with details defining the dimple pattern of the cover that will be produced. The upper and lower mold cavities are joined together under sufficient heat and pressure. The polyurethane material in the cavities encapsulates the ball subassembly and forms the cover of the ball.

After the golf balls have been removed from the mold, they may be subjected to finishing steps including flash-trimming, surface-treatment, marking, and application of coatings. Optical brighteners can be included in the cover stock material used to make the cover layer, in primer coatings, in paints, and in topcoat composition. When applied to the exterior of a golf ball, optical brighteners enhance the whiteness and/or brightness of such balls. Clear topcoats are often applied to the cover of the golf ball. The topcoats protect the ball any underlying clear or pigmented layers. The topcoats also protect any trademarks, tradenames logos, and other indicia printed on the ball. The topcoats normally have a high gloss finish and help provide the ball with an aesthetically pleasing appearance.

For example, in Proudfit, U.S. Pat. No. 5,000,458, a transparent primer coat is applied over the cover of a golf ball, and a transparent outermost clear coat is applied over the primer coat. The primer coat contains an optical brightener. In Hatch et al., U.S. Pat. No. 5,820,491 describes a polyurethane topcoat composition that can be applied to golf balls having polyurethane covers. The topcoat may contain optical brighteners. According to the '491 Patent, the topcoat has improved abrasion resistance, mar resistance and detergent resistance. In Wu, U.S. Pat. No. 6,528,578, thermoplastic or thermosetting polyurethanes and ionomers are described as being suitable materials for making outer cover layers. The cover layer composition contains ultraviolet (UV) light absorbers and optical brighteners. In Chavan, U.S. Pat. No. 9,962,577, a polyurethane coating containing optical brighteners is applied to the golf ball cover. Thermoplastic and thermoset polyurethanes can be used to make the golf ball cover.

Although topcoats for golf balls have been used over the years, there are drawbacks with using some topcoat compositions. For example, in some instances, if the topcoat contains a relatively high concentration of optical brighteners, this can cause discoloration problems in the cover layer of the ball. The ball may develop a yellowish tint. In view of some of the drawbacks with some conventional topcoats, it would be desirable to have new, cost-effective, efficient topcoat composition that can be used to produce golf balls with desirable physical and playing performance properties. The present invention provides new topcoat formulations and new methods for making thermoplastic polyurethane covers for golf balls having a topcoat composition with many advantageous features and benefits. The invention also includes the resulting golf balls having good physical and playing performance properties.

SUMMARY OF THE INVENTION

The present invention generally relates to golf balls having covers made of thermoplastic polyurethane compositions. The invention includes methods for applying polyurethane top coatings to the thermoplastic polyurethane cover. In one embodiment, a method for forming a coated golf ball comprises the steps of: a) providing a golf ball comprising at least one core layer and an outer cover layer, wherein the outer cover layer is formed from a thermoplastic polyurethane composition; and b) applying a polyurethane

coating to the outer cover layer, the coating comprising an optical brightener in a concentration of about 0.01 to about 0.20 weight %. The wet weight of the polyurethane coating is in the range of about 0.20 g to about 0.42 g. In a particularly preferred example, the optical brightener is in a concentration of about 0.1 to about 1.0 wt. %, and is selected from the group consisting of triazine-stilbenes (di-, tetra-, or hexa-sulfonated); coumarins; imidazolines; diazoles; triazoles; benzoxazolines; and biphenyl-stilbenes; and mixtures thereof.

More particularly, the polyurethane coating can be produced by mixing a Part A component and Part B component, wherein the Part A component comprises about polyol in an amount of about 30 to about 60 weight %; catalyst in an amount of about 0.1 to about 5.0 weight %); solvent in an amount of about 40 to about 70 wt. %); fluorosurfactant in an amount of about 0.1 to about 3.0 wt. %; ultraviolet light stabilizers in an amount of about 0.1 to about 5.0 wt. %); and the Part B component comprises polyisocyanate in an amount of about 10 to about 100 wt. % polyisocyanate and solvent in an amount of about 0 to about 90 wt. %.

Suitable isocyanates include, for example, those selected from the group consisting of toluene 2,4-diisocyanate (TDI), toluene 2,6-diisocyanate (TDI), 4,4'-dicyclohexylmethane diisocyanate (H<sub>12</sub> MDI), isophorone diisocyanate (IPDI), meta-tetramethylxylylene diisocyanate (TMXDI), trans-cyclohexane diisocyanate (CHDI), and homopolymers and copolymers and blends thereof. Suitable solvents include, for example, those selected from the group consisting of ketones, acetates, and mixtures thereof.

The methods of this invention can be used to make thin outer cover layers. In one example, the outer cover has a thickness in the range of about 0.010 to about 0.050 inches, and a hardness in the range of about 20 to about 59 Shore D. Multi-piece golf balls having inner cores, outer cores, inner covers, and intermediate layers can be made.

IN another embodiment, the method comprises the steps of: i) providing a golf ball comprising at least one core layer and an outer cover layer, wherein the outer cover layer is formed from a thermoplastic polyurethane composition; ii) applying a first polyurethane coating comprising unreacted isocyanate groups and having an isocyanate index of at least about 115 to the outer cover layer; iii) treating the golf ball with heat; and iv) applying a second polyurethane coating to the outer cover of the golf ball, the second polyurethane coating comprising an optical brightener in a concentration of about 0.01 to about 0.20 weight %, to form a coated golf ball.

invention also encompasses golf balls made by the above-described methods. The golf balls having the topcoat composition of this invention have optimum properties. The balls have a sufficient amount of optical brighteners to provide the desired brightness to the golf ball; and yet at the same time, the ball does not suffer from discoloration problems such as a greening effect when exposed to sunlight. Furthermore, the topcoat of this invention has good uniformity and impact-durability.

#### BRIEF DESCRIPTION OF THE DRAWINGS

The novel features that are characteristic of the present invention are set forth in the appended claims. However, the preferred embodiments of the invention, together with further objects and attendant advantages, are best understood by reference to the following detailed description in connection with the accompanying drawings in which:

FIG. 1 is a perspective view of a dimpled golf ball made in accordance with the present invention;

FIG. 2 is a cross-sectional view of a two-piece golf ball having an inner core and outer cover made in accordance with the present invention;

FIG. 3 is a cross-sectional view of another two-piece golf ball having an inner core and outer cover made in accordance with the present invention;

FIG. 4 is a cross-sectional view of a three-piece golf ball having an inner core, outer core, and outer cover made in accordance with the present invention;

FIG. 5 is a partial cut-away perspective view of a three-piece golf ball having an inner core, outer core, and outer cover made in accordance with the present invention; and

FIG. 6 is a cross-sectional view of a four-piece golf ball having an inner core, outer core, inner cover, and outer cover made in accordance with the present invention.

#### DETAILED DESCRIPTION OF THE INVENTION

The present invention relates generally to golf balls having covers made of thermoplastic polyurethane (TPU) compositions. Different polyurethane primer and top-coats are applied to the polyurethane outer cover in accordance with this invention. The invention also includes the finished golf balls made from these coating applications.

Golf balls having various constructions may be made in accordance with this invention. For example, golf balls having three piece, four-piece, and five-piece constructions with single or multi-layered cover materials may be made. Representative illustrations of such golf ball constructions are provided and discussed further below. The term, "layer" as used herein means generally any spherical portion of the golf ball. More particularly, in one version, a two-piece golf ball containing a core and having a surrounding cover is made. Three-piece golf balls containing a dual-layered core and single-layered cover also can be made. The dual-core includes an inner core (center) and surrounding outer core layer. In another version, a four-piece golf ball containing a dual-core and dual-cover (inner cover and outer cover layers) is made. In yet another construction, a four-piece or five-piece golf ball containing a dual-core; casing layer(s); and cover layer(s) may be made. As used herein, the term, "casing layer" means a layer of the ball disposed between the multi-layered core sub-assembly and cover. The casing layer also may be referred to as a mantle or intermediate layer. The diameter and thickness of the different layers along with properties such as hardness and compression may vary depending upon the construction and desired playing performance properties of the golf ball as discussed further below.

##### Core Structure

The golf ball may contain a single- or multi-layered core.

In one preferred embodiment, at least one of the core layers is formed of a rubber composition comprising polybutadiene rubber material. More particularly, in one version, the ball contains a single inner core formed of the polybutadiene rubber composition. In a second version, the ball contains a dual-core comprising an inner core (center) and surrounding outer core layer.

In one version, the core is formed of a rubber composition comprising a rubber material such as, for example, polybutadiene, ethylene-propylene rubber, ethylene-propylene-diene rubber, polyisoprene, styrene-butadiene rubber, poly-alkenamers, butyl rubber, halobutyl rubber, or polystyrene elastomers. For example, polybutadiene rubber composi-

tions may be used to form the inner core (center) and surrounding outer core layer in a dual-layer construction. In another version, the core may be formed from an ionomer composition comprising an ethylene acid copolymer containing acid groups such that greater than 70% of the acid groups are neutralized. These highly neutralized polymers (HNPs) also may be used to form at least one core layer in a multi-layered core construction. For example, a polybutadiene rubber composition may be used to form the center and a HNP composition may be used to form the outer core. Such rubber and HNP compositions are discussed in further detail below.

In general, polybutadiene is a homopolymer of 1, 3-butadiene. The double bonds in the 1, 3-butadiene monomer are attacked by catalysts to grow the polymer chain and form a polybutadiene polymer having a desired molecular weight. Any suitable catalyst may be used to synthesize the polybutadiene rubber depending upon the desired properties. Normally, a transition metal complex (for example, neodymium, nickel, or cobalt) or an alkyl metal such as alkyl-lithium is used as a catalyst. Other catalysts include, but are not limited to, aluminum, boron, lithium, titanium, and combinations thereof. The catalysts produce polybutadiene rubbers having different chemical structures. In a cis-bond configuration, the main internal polymer chain of the polybutadiene appears on the same side of the carbon-carbon double bond contained in the polybutadiene. In a trans-bond configuration, the main internal polymer chain is on opposite sides of the internal carbon-carbon double bond in the polybutadiene. The polybutadiene rubber can have various combinations of cis- and trans-bond structures. A preferred polybutadiene rubber has a 1,4 cis-bond content of at least 40%, preferably greater than 80%, and more preferably greater than 90%. In general, polybutadiene rubbers having a high 1,4 cis-bond content have high tensile strength. The polybutadiene rubber may have a relatively high or low Mooney viscosity.

Examples of commercially-available polybutadiene rubbers that can be used in accordance with this invention, include, but are not limited to, BR 01 and BR 1220, available from BST Elastomers of Bangkok, Thailand; SE BR 1220LA and SE BR 1203, available from DOW Chemical Co of Midland, Mich.; BUDENE 1207, 1207s, 1208, and 1280 available from Goodyear, Inc of Akron, Ohio; BR 01, 51 and 730, available from Japan Synthetic Rubber (JSR) of Tokyo, Japan; BUNA CB 21, CB 22, CB 23, CB 24, CB 25, CB 29 MES, CB 60, CB Nd 60, CB 55 NF, CB 70 B, CB KA 8967, and CB 1221, available from Lanxess Corp. of Pittsburgh, Pa.; BR1208, available from LG Chemical of Seoul, South Korea; UBEPOL BR130B, BR150, BR150B, BR150L, BR230, BR360L, BR710, and VCR617, available from UBE Industries, Ltd. of Tokyo, Japan; EUROPRENE NEO-CIS BR 60, INTENE 60 AF and P30AF, and EUROPRENE BR HV80, available from Polimeri Europa of Rome, Italy; AFIDENE 50 and NEODENE BR40, BR45, BR50 and BR60, available from Karbochem (PTY) Ltd. of Bruma, South Africa; KBR 01, NdBr 40, NdBr-45, NdBr 60, KBR 710S, KBR 710H, and KBR 750, available from Kumho Petrochemical Co., Ltd. Of Seoul, South Korea; and DIENE 55NF, 70AC, and 320 AC, available from Firestone Polymers of Akron, Ohio.

To form the core, the polybutadiene rubber is used in an amount of at least about 5% by weight based on total weight of composition and is generally present in an amount of about 5% to about 100%, or an amount within a range having a lower limit of 5% or 10% or 20% or 30% or 40% or 50% and an upper limit of 55% or 60% or 70% or 80%

or 90% or 95% or 100%. In general, the concentration of polybutadiene rubber is about 45 to about 95 weight percent. Preferably, the rubber material used to form the core layer comprises at least 50% by weight, and more preferably at least 70% by weight, polybutadiene rubber.

The rubber compositions of this invention may be cured, either by pre-blending or post-blending, using conventional curing processes. Suitable curing processes include, for example, peroxide-curing, sulfur-curing, high-energy radiation, and combinations thereof. Preferably, the rubber composition contains a free-radical initiator selected from organic peroxides, high energy radiation sources capable of generating free-radicals, and combinations thereof. In one preferred version, the rubber composition is peroxide-cured. Suitable organic peroxides include, but are not limited to, dicumyl peroxide; n-butyl-4,4-di(t-butylperoxy) valerate; 1,1-di(t-butylperoxy)3,3,5-trimethylcyclohexane; 2,5-dimethyl-2,5-di(t-butylperoxy)hexane; di-t-butyl peroxide; di-t-amyl peroxide; t-butyl peroxide; t-butyl cumyl peroxide; 2,5-dimethyl-2,5-di(t-butylperoxy)hexyne-3; di(2-t-butylperoxyisopropyl)benzene; dilauroyl peroxide; dibenzoyl peroxide; t-butyl hydroperoxide; and combinations thereof. In a particular embodiment, the free radical initiator is dicumyl peroxide, including, but not limited to Perkadox® BC, commercially available from Akzo Nobel. Peroxide free-radical initiators are generally present in the rubber composition in an amount of at least 0.05 parts by weight per 100 parts of the total rubber, or an amount within the range having a lower limit of 0.05 parts or 0.1 parts or 1 part or 1.25 parts or 1.5 parts or 2.5 parts or 5 parts by weight per 100 parts of the total rubbers, and an upper limit of 2.5 parts or 3 parts or 5 parts or 6 parts or 10 parts or 15 parts by weight per 100 parts of the total rubber. Concentrations are in parts per hundred (phr) unless otherwise indicated. As used herein, the term, "parts per hundred," also known as "phr" or "pph" is defined as the number of parts by weight of a particular component present in a mixture, relative to 100 parts by weight of the polymer component. Mathematically, this can be expressed as the weight of an ingredient divided by the total weight of the polymer, multiplied by a factor of 100.

The rubber compositions preferably include a reactive cross-linking co-agent. Suitable co-agents include, but are not limited to, metal salts of unsaturated carboxylic acids having from 3 to 8 carbon atoms; unsaturated vinyl compounds and polyfunctional monomers (e.g., trimethylolpropane trimethacrylate); phenylene bismaleimide; and combinations thereof. Particular examples of suitable metal salts include, but are not limited to, one or more metal salts of acrylates, diacrylates, methacrylates, and dimethacrylates, wherein the metal is selected from magnesium, calcium, zinc, aluminum, lithium, and nickel. In a particular embodiment, the co-agent is selected from zinc salts of acrylates, diacrylates, methacrylates, and dimethacrylates. In another particular embodiment, the agent is zinc diacrylate (ZDA). When the co-agent is zinc diacrylate and/or zinc dimethacrylate, the co-agent is typically included in the rubber composition in an amount within the range having a lower limit of 1 or 5 or 10 or 15 or 19 or 20 parts by weight per 100 parts of the total rubber, and an upper limit of 24 or 25 or 30 or 35 or 40 or 45 or 50 or 60 parts by weight per 100 parts of the base rubber.

Radical scavengers such as a halogenated organosulfur or metal salt thereof, organic disulfide, or inorganic disulfide compounds may be added to the rubber composition. These compounds also may function as "soft and fast agents." As used herein, "soft and fast agent" means any compound or

a blend thereof that is capable of making a core: 1) softer (having a lower compression) at a constant “coefficient of restitution” (COR); and/or 2) faster (having a higher COR at equal compression), when compared to a core equivalently prepared without a soft and fast agent. Preferred halogenated organosulfur compounds include, but are not limited to, pentachlorothiophenol (PCTP) and salts of PCTP such as zinc pentachlorothiophenol (ZnPCTP). Using PCTP and ZnPCTP in golf ball inner cores helps produce softer and faster inner cores. The PCTP and ZnPCTP compounds help increase the resiliency and the coefficient of restitution of the core. In a particular embodiment, the soft and fast agent is selected from ZnPCTP, PCTP, ditolyl disulfide, diphenyl disulfide, dixylyl disulfide, 2-nitroresorcinol, and combinations thereof.

The rubber compositions of the present invention also may include “fillers,” which are added to adjust the density and/or specific gravity of the material. Suitable fillers include, but are not limited to, polymeric or mineral fillers, metal fillers, metal alloy fillers, metal oxide fillers and carbonaceous fillers. The fillers can be in any suitable form including, but not limited to, flakes, fibers, whiskers, fibrils, plates, particles, and powders. Rubber grind, which is ground, recycled rubber material (for example, ground to about 30 mesh particle size) obtained from discarded rubber golf ball cores, also can be used as a filler. The amount and type of fillers utilized are governed by the amount and weight of other ingredients in the golf ball, since a maximum golf ball weight of 45.93 g (1.62 ounces) has been established by the United States Golf Association (USGA).

Suitable polymeric or mineral fillers that may be added to the rubber composition include, for example, precipitated hydrated silica, clay, talc, asbestos, glass fibers, aramid fibers, mica, calcium metasilicate, barium sulfate, zinc sulfide, lithopone, silicates, silicon carbide, tungsten carbide, diatomaceous earth, polyvinyl chloride, carbonates such as calcium carbonate and magnesium carbonate. Suitable metal fillers include titanium, tungsten, aluminum, bismuth, nickel, molybdenum, iron, lead, copper, boron, cobalt, beryllium, zinc, and tin. Suitable metal alloys include steel, brass, bronze, boron carbide whiskers, and tungsten carbide whiskers. Suitable metal oxide fillers include zinc oxide, iron oxide, aluminum oxide, titanium oxide, magnesium oxide, and zirconium oxide. Suitable particulate carbonaceous fillers include graphite, carbon black, cotton flock, natural bitumen, cellulose flock, and leather fiber. Micro balloon fillers such as glass and ceramic, and fly ash fillers can also be used. In a particular aspect of this embodiment, the rubber composition includes filler(s) selected from carbon black, nanoclays (e.g., Cloisite® and Nanofil® nanoclays, commercially available from Southern Clay Products, Inc., and Nanomax® and Nanomer® nanoclays, commercially available from Nanocor, Inc.), talc (e.g., Luzenac HAR® high aspect ratio talcs, commercially available from Luzenac America, Inc.), glass (e.g., glass flake, milled glass, and microglass), mica and mica-based pigments (e.g., Iridin® pearl luster pigments, commercially available from The Merck Group), and combinations thereof. In a particular embodiment, the rubber composition is modified with organic fiber micropulp.

In addition, the rubber compositions may include antioxidants to prevent the breakdown of the elastomers. Also, processing aids such as high molecular weight organic acids and salts thereof, may be added to the composition. In a particular embodiment, the total amount of additive(s) and filler(s) present in the rubber composition is 15 wt % or less, or 12 wt % or less, or 10 wt % or less, or 9 wt % or less, or

6 wt % or less, or 5 wt % or less, or 4 wt % or less, or 3 wt % or less, based on the total weight of the rubber composition.

The polybutadiene rubber material (base rubber) may be 5 blended with other elastomers in accordance with this invention. Other elastomers include, but are not limited to, polybutadiene, polyisoprene, ethylene propylene rubber (“EPR”), styrene-butadiene rubber, styrenic block copolymer rubbers (such as “SI”, “SIS”, “SB”, “SBS”, “SIBS”, and the like, 10 where “S” is styrene, “I” is isobutylene, and “B” is butadiene), polyalkenamers such as, for example, polyoctenamer, butyl rubber, halobutyl rubber, polystyrene elastomers, polyethylene elastomers, polyurethane elastomers, polyurea elastomers, metallocene-catalyzed elastomers and plasto- 15 polymers, copolymers of isobutylene and p-alkylstyrene, halogenated copolymers of isobutylene and p-alkylstyrene, copolymers of butadiene with acrylonitrile, polychloroprene, alkyl acrylate rubber, chlorinated isoprene rubber, acrylonitrile chlorinated isoprene rubber, and combinations 20 of two or more thereof.

The polymers, free-radical initiators, filler, cross-linking agents, and any other materials used in forming either the golf ball center or any portion of the core, in accordance with 25 invention, may be combined to form a mixture by any type of mixing known to one of ordinary skill in the art. Suitable types of mixing include single pass and multi-pass mixing, and the like. The cross-linking agent, and any other optional additives used to modify the characteristics of the golf ball center or additional layer(s), may similarly be combined by 30 any type of mixing. A single-pass mixing process where ingredients are added sequentially is preferred, as this type of mixing tends to increase efficiency and reduce costs for the process. The preferred mixing cycle is single step wherein the polymer, cis-to-trans catalyst, filler, zinc di- 35 crylate, and peroxide are added in sequence.

In one preferred embodiment, the entire core or at least one core layer in a multi-layered structure is formed of a 40 rubber composition comprising a material selected from the group of natural and synthetic rubbers including, but not limited to, polybutadiene, polyisoprene, ethylene propylene rubber (“EPR”), ethylene-propylene-diene (“EPDM”) rubber, styrene-butadiene rubber, styrenic block copolymer rubbers (such as “SI”, “SIS”, “SB”, “SBS”, “SIBS”, and the like, where “S” is styrene, “I” is isobutylene, and “B” is butadiene), polyalkenamers such as, for example, polyoctenamer, butyl rubber, halobutyl rubber, polystyrene elastomers, polyethylene elastomers, polyurethane elastomers, polyurea elastomers, metallocene-catalyzed elastomers and plasto- 45 polymers, copolymers of isobutylene and p-alkylstyrene, halogenated copolymers of isobutylene and p-alkylstyrene, copolymers of butadiene with acrylonitrile, polychloroprene, alkyl acrylate rubber, chlorinated isoprene rubber, acrylonitrile chlorinated isoprene rubber, and combinations 50 of two or more thereof.

55 As discussed above, single and multi-layered cores can be made in accordance with this invention. In two-layered cores, a thermoset material such as, for example, thermoset rubber, can be used to make the outer core layer or a thermoplastic material such as, for example, ethylene acid 60 copolymer containing acid groups that are at least partially or fully neutralized can be used to make the outer core layer. Suitable ionomer compositions include partially-neutralized ionomers and highly-neutralized ionomers (HNPs), including ionomers formed from blends of two or more partially-neutralized ionomers, blends of two or more highly-neutralized ionomers, and blends of one or more partially-neutralized ionomers with one or more highly-neutralized

ionomers. Suitable ethylene acid copolymer ionomers and other thermoplastics that can be used to form the core layer(s) are the same materials that can be used to make an inner cover layer as discussed further below.

In another example, multi-layered cores having an inner core, intermediate core layer, and outer core layer, wherein the intermediate core layer is disposed between the intermediate and outer core layers may be prepared in accordance with this invention. More particularly, as discussed above, the inner core may be constructed from a thermoplastic or thermoset composition, such as thermoset rubber. Meanwhile, the intermediate and outer core layers also may be formed from thermoset or thermoplastic materials. Suitable thermoset and thermoplastic compositions that may be used to form the intermediate/outer core layers are discussed above. For example, each of the intermediate and outer core layers may be formed from a thermoset rubber composition. Thus, the intermediate core layer may be formed from a first thermoset rubber composition; and the outer core layer may be formed from a second thermoset rubber composition. In another embodiment, the intermediate core layer is formed from a thermoset composition; and the outer core layer is formed from a thermoplastic composition. In a third embodiment, the intermediate core layer is formed from a thermoplastic composition; and the outer core layer is formed from a thermoset composition. Finally, in a fourth embodiment, the intermediate core layer is formed from a first thermoplastic composition; and the outer core layer is formed from a second thermoplastic composition.

In a particular embodiment, the core includes at least one additional thermoplastic intermediate core layer formed from a composition comprising an ionomer selected from DuPont® HPF ESX 367, HPF 1000, HPF 2000, HPF AD1035, HPF AD1035 Soft, HPF AD1040, and AD1172 ionomers, commercially available from E. I. du Pont de Nemours and Company. The coefficient of restitution (“COR”), compression, and surface hardness of each of these materials, as measured on 1.55" injection molded spheres aged two weeks at 23° C./50% RH, are given in Table 1 below.

TABLE 1

| Example         | Solid Sphere COR | Solid Sphere Compression | Solid Sphere Shore D Surface Hardness |
|-----------------|------------------|--------------------------|---------------------------------------|
| HPF 1000        | 0.830            | 115                      | 54                                    |
| HPF 2000        | 0.860            | 90                       | 47                                    |
| HPF AD1035      | 0.820            | 63                       | 42                                    |
| HPF AD1035 Soft | 0.780            | 33                       | 35                                    |
| HPF AD 1040     | 0.855            | 135                      | 60                                    |
| HPF AD1172      | 0.800            | 32                       | 37                                    |

#### Cover Layer Structure

The golf balls of this invention further include an outer cover layer preferably made of a thermoplastic polyurethane composition. In general, polyurethanes contain urethane linkages formed by reacting an isocyanate group ( $-\text{N}=\text{C}=\text{O}$ ) with a hydroxyl group (OH). The polyurethanes are produced by the reaction of a multi-functional isocyanate ( $\text{NCO}-\text{R}-\text{NCO}$ ) with a long-chain polyol having terminal hydroxyl groups (OH—OH) in the presence of a catalyst and other additives. The chain length of the polyurethane prepolymer is extended by reacting it with short-chain diols (OH—R'—OH). The resulting polyurethane has elastomeric properties because of its “hard” and “soft” segments, which are covalently bonded together. This

phase separation occurs because the mainly non-polar, low melting soft segments are incompatible with the polar, high melting hard segments. The hard segments, which are formed by the reaction of the diisocyanate and low molecular weight chain-extending diol, are relatively stiff and immobile. The soft segments, which are formed by the reaction of the diisocyanate and long chain diol, are relatively flexible and mobile. Because the hard segments are covalently coupled to the soft segments, they inhibit plastic flow of the polymer chains, thus creating elastomeric resiliency.

By the term, “isocyanate compound” as used herein, it is meant any aliphatic or aromatic isocyanate containing two or more isocyanate functional groups. The isocyanate compounds can be monomers or monomeric units, because they can be polymerized to produce polymeric isocyanates containing two or more monomeric isocyanate repeat units. The isocyanate compound may have any suitable backbone chain structure including saturated or unsaturated, and linear, branched, or cyclic. These isocyanate compounds also can be referred to as polyisocyanates or multi-functional isocyanates. By the term, “polyamine” as used herein, it is meant any aliphatic or aromatic compound containing two or more primary or secondary amine functional groups. The polyamine compound may have any suitable backbone chain structure including saturated or unsaturated, and linear, branched, or cyclic. The term “polyamine” may be used interchangeably with amine-terminated component. These polyamines also can be referred to as amine compounds or multi-functional amines. By the term, “polyol” as used herein, it is meant any aliphatic or aromatic compound containing two or more hydroxyl functional groups. The term “polyol” may be used interchangeably with hydroxy-terminated component. By the term, “polyimine compound”, it is meant it is meant any aliphatic or aromatic compound containing two or more imine functional groups. These polyimines also can be referred to as imine compounds or multi-functional imines.

Thermoplastic polyurethanes have minimal cross-linking; any bonding in the polymer network is primarily through hydrogen bonding or other physical mechanism. Because of their lower level of cross-linking, thermoplastic polyurethanes are relatively flexible. The cross-linking bonds in thermoplastic polyurethanes can be reversibly broken by increasing temperature such as during molding or extrusion. That is, the thermoplastic material softens when exposed to heat and returns to its original condition when cooled. On the other hand, thermoset polyurethanes become irreversibly set when they are cured. The cross-linking bonds are irreversibly set and are not broken when exposed to heat. Thus, thermoset polyurethanes, which typically have a high level of cross-linking, are relatively rigid.

Commercially-available examples of suitable thermoplastic polyurethanes that can be used in accordance with this invention include TPUs sold under the tradenames of Texin® 250, Texin® 255, Texin® 260, Texin® 270, Texin®950U, Texin® 970U, Texin®1049, Texin® 990DP7-1191, Texin® DP7-1202, Texin®990R, Texin®993, Texin® DP7-1049, Texin® 3203, Texin® 4203, Texin® 4206, Texin® 4210, Texin® 4215, and Texin® 3215, each commercially available from Covestro LLC, Pittsburgh Pa.; Estane® 50 DT3, Estane®58212, Estane®55DT3, Estane®58887, Estane® EZ14-23A, Estane® ETE 50DT3, each commercially available from Lubrizol Company of Cleveland, Ohio; and Elastollan® WY1149, Elastollan®1154D53, Elastollan®1180A, Elastollan®1190A, Elastollan®1195A,

## 11

Elastollan®1185AW, Elastollan®1175AW, each commercially available from BASF; Desmopan® 453, commercially available from Bayer of Pittsburgh, Pa., and the E-Series TPUs, such as D 60 E 4024 commercially available from Huntsman Polyurethanes of Germany.

Aromatic polyurethanes can be prepared in accordance with this invention and these materials are preferably formed by reacting an aromatic diisocyanate with a polyol. Suitable aromatic diisocyanates that may be used in accordance with this invention include, for example, toluene 2,4-diisocyanate (TDI), toluene 2,6-diisocyanate (TDI), 4,4'-methylene diphenyl diisocyanate (MDI), 2,4'-methylene diphenyl diisocyanate (MDI), polymeric methylene diphenyl diisocyanate (PMDI), p-phenylene diisocyanate (PPDI), m-phenylene diisocyanate (PDI), naphthalene 1,5-diisocyanate (NDI), naphthalene 2,4-diisocyanate (NDI), p-xylene diisocyanate (XDI), and homopolymers and copolymers and blends thereof. The aromatic isocyanates are able to react with the hydroxyl or amine compounds and form a durable and tough polymer having a high melting point. The resulting polyurethane generally has good mechanical strength and cut/shear-resistance.

Aliphatic polyurethanes also can be prepared in accordance with this invention and these materials are preferably formed by reacting an aliphatic diisocyanate with a polyol. Suitable aliphatic diisocyanates that may be used in accordance with this invention include, for example, isophorone diisocyanate (IPDI), 1,6-hexamethylene diisocyanate (HDI), 4,4'-dicyclohexylmethane diisocyanate ("H<sub>12</sub> MDI"), meta-tetramethylxylylene diisocyanate (TMXDI), trans-cyclohexane diisocyanate (CHDI), and homopolymers and copolymers and blends thereof. Particularly suitable multi-functional isocyanates include trimers of HDI or H<sub>12</sub> MDI, oligomers, or other derivatives thereof. The resulting polyurethane generally has good light and thermal stability.

Any polyol available to one of ordinary skill in the art is suitable for use according to the invention. Exemplary polyols include, but are not limited to, polyether polyols, hydroxy-terminated polybutadiene (including partially/fully hydrogenated derivatives), polyester polyols, polycaprolactone polyols, and polycarbonate polyols. In one preferred embodiment, the polyol includes polyether polyol. Examples include, but are not limited to, polytetramethylene ether glycol (PTMEG) which is particularly preferred, polyethylene propylene glycol, polyoxypolyethylene glycol, and mixtures thereof. The hydrocarbon chain can have saturated or unsaturated bonds and substituted or unsubstituted aromatic and cyclic groups.

In another embodiment, polyester polyols are included in the polyurethane material. Suitable polyester polyols include, but are not limited to, polyethylene adipate glycol; polybutylene adipate glycol; polyethylene propylene adipate glycol; o-phthalate-1,6-hexanediol; poly(hexamethylene adipate) glycol; and mixtures thereof. The hydrocarbon chain can have saturated or unsaturated bonds, or substituted or unsubstituted aromatic and cyclic groups. In still another embodiment, polycaprolactone polyols are included in the materials of the invention. Suitable polycaprolactone polyols include, but are not limited to: 1,6-hexanediol-initiated polycaprolactone, diethylene glycol initiated polycaprolactone, trimethylol propane initiated polycaprolactone, neopentyl glycol initiated polycaprolactone, 1,4-butanediol-initiated polycaprolactone, and mixtures thereof. The hydrocarbon chain can have saturated or unsaturated bonds, or substituted or unsubstituted aromatic and cyclic groups. In yet another embodiment, polycarbonate polyols are included in the polyurethane material of the invention.

## 12

Suitable polycarbonates include, but are not limited to, polyphthalate carbonate and poly(hexamethylene carbonate) glycol. The hydrocarbon chain can have saturated or unsaturated bonds, or substituted or unsubstituted aromatic and cyclic groups. In one embodiment, the molecular weight of the polyol is from about 200 to about 4000.

There are two basic techniques that can be used to make the polyurethanes: a) one-shot technique, and b) prepolymer technique. In the one-shot technique, the diisocyanate, 10 polyol, and hydroxyl-terminated chain-extender (curing agent) are reacted in one step. On the other hand, the prepolymer technique involves a first reaction between the diisocyanate and polyol compounds to produce a polyurethane prepolymer, and a subsequent reaction between the 15 prepolymer and hydroxyl-terminated chain-extender. As a result of the reaction between the isocyanate and polyol compounds, there will be some unreacted NCO groups in the polyurethane prepolymer. The prepolymer should have less than 14% unreacted NCO groups. Preferably, the prepolymer has no greater than 8.5% unreacted NCO groups, more 20 preferably from 2.5% to 8%, and most preferably from 5.0% to 8.0% unreacted NCO groups. As the weight percent of unreacted isocyanate groups increases, the hardness of the composition also generally increases.

25 Either the one-shot or prepolymer method may be employed to produce the polyurethane compositions of the invention. In one embodiment, the one-shot method is used, wherein the isocyanate compound is added to a reaction vessel and then a curative mixture comprising the polyol and 30 curing agent is added to the reaction vessel. The components are mixed together so that the molar ratio of isocyanate groups to hydroxyl groups is preferably in the range of about 1.00:1.00 to about 1.10:1.00. In a second embodiment, the prepolymer method is used. In general, the prepolymer 35 technique is preferred because it provides better control of the chemical reaction. The prepolymer method provides a more homogeneous mixture resulting in a more consistent polymer composition. The one-shot method results in a mixture that is inhomogeneous (more random) and affords 40 the manufacturer less control over the molecular structure of the resultant composition.

The polyurethane compositions can be formed by chain-extending the polyurethane prepolymer with a single chain-extender or blend of chain-extenders as described further 45 below. As discussed above, the polyurethane prepolymer can be chain-extended by reacting it with a single chain-extender or blend of chain-extenders. In general, the prepolymer can be reacted with hydroxyl-terminated curing agents, amine-terminated curing agents, and mixtures thereof. The curing agents extend the chain length of the prepolymer and build-up its molecular weight. In general, thermoplastic 50 polyurethane compositions are typically formed by reacting the isocyanate blend and polyols at a 1:1 stoichiometric ratio. Thermoset compositions, on the other hand, are cross-linked polymers and are typically produced from the reaction 55 of the isocyanate blend and polyols at normally a 1.05:1 stoichiometric ratio

A catalyst may be employed to promote the reaction 60 between the isocyanate and polyol compounds for producing the prepolymer or between prepolymer and chain-extender during the chain-extending step. Preferably, the catalyst is added to the reactants before producing the prepolymer. Suitable catalysts include, but are not limited to, bismuth catalyst; zinc octoate; stannous octoate; tin catalysts such as 65 bis-butylin dilaurate, bis-butylin diacetate, stannous octoate; tin (II) chloride, tin (IV) chloride, bis-butylin dimethoxide, dimethyl-bis[1-oxonenedecyl]oxy]stannane, di-

n-octyltin bis-isoctyl mercaptoacetate; amine catalysts such as triethylenediamine, triethylamine, and tributylamine; organic acids such as oleic acid and acetic acid; delayed catalysts; and mixtures thereof. The catalyst is preferably added in an amount sufficient to catalyze the reaction of the components in the reactive mixture. In one embodiment, the catalyst is present in an amount from about 0.001 percent to about 1 percent, and preferably 0.1 to 0.5 percent, by weight of the composition.

The hydroxyl chain-extending (curing) agents are preferably selected from the group consisting of ethylene glycol; diethylene glycol; polyethylene glycol; propylene glycol; 2-methyl-1,3-propanediol; 2-methyl-1,4-butanediol; monoethanolamine; diethanolamine; triethanolamine; monoiso-propanolamine; diisopropanolamine; dipropylene glycol; polypropylene glycol; 1,2-butanediol; 1,3-butanediol; 1,4-butanediol; 2,3-butanediol; 2,3-dimethyl-2,3-butanediol; trimethylolpropane; cyclohexyldimethylol; triisopropanolamine; N,N,N',N'-tetra-(2-hydroxypropyl)-ethylene diamine; diethylene glycol bis-(aminopropyl) ether; 1,5-pentanediol; 1,6-hexanediol; 1,3-bis-(2-hydroxyethoxy) cyclohexane; 1,4-cyclohexyldimethylol; 1,3-bis-[2-(2-hydroxyethoxy) ethoxy]cyclohexane; 1,3-bis-{2-[2-(2-hydroxyethoxy) ethoxy]ethoxy}cyclohexane; trimethylolpropane; polytetramethylene ether glycol (PTMEG), preferably having a molecular weight from about 250 to about 3900; and mixtures thereof.

Suitable amine chain-extending (curing) agents that can be used in chain-extending the polyurethane prepolymer include, but are not limited to, unsaturated diamines such as 4,4'-diamino-diphenylmethane (i.e., 4,4'-methylene-dianiline or "MDA"), m-phenylenediamine, p-phenylenediamine, 1,2- or 1,4-bis(sec-butylamino)benzene, 3,5-diethyl-(2,4- or 2,6-) toluediamine or "DETDA", 3,5-dimethylthio-(2,4- or 2,6-) toluediamine, 3,5-diethylthio-(2,4- or 2,6-) toluediamine, 3,3'-dimethyl-4,4'-diamino-diphenylmethane, 3,3'-diethyl-5,5'-dimethyl 4,4'-diamino-diphenylmethane (i.e., 4,4'-methylene-bis(2-ethyl-6-methylbenzeneamine)), 3,3'-dichloro-4,4'-diamino-diphenylmethane (i.e., 4,4'-methylene-bis(2-chloroaniline) or "MOCA"), 3,3',5,5'-tetraethyl-4,4'-diamino-diphenylmethane (i.e., 4,4'-methylene-bis(2,6-diethylaniline), 2,2'-dichloro-3,3',5,5'-tetraethyl-4,4'-diamino-diphenylmethane (i.e., 4,4'-methylene-bis(3-chloro-2,6-diethylenaniline) or "MCDEA"), 3,3'-diethyl-5,5'-dichloro-4,4'-diamino-diphenylmethane, or "MDEA"), 3,3'-dichloro-2,2',6,6'-tetraethyl-4,4'-diamino-diphenylmethane, 3,3'-dichloro-4,4'-diamino-diphenylmethane, 4,4'-methylene-bis(2,3-dichloroaniline) (i.e., 2,2',3,3'-tetrachloro-4,4'-diamino-diphenylmethane or "MDCA"); and mixtures thereof. One particularly suitable amine-terminated chain-extending agent is Ethacure 300<sup>TM</sup> (dimethylthiotoluediamine or a mixture of 2,6-diamino-3,5-dimethylthiotoluene and 2,4-diamino-3,5-dimethylthiotoluene.) The amine curing agents used as chain extenders normally have a cyclic structure and a low molecular weight (250 or less).

When the polyurethane prepolymer is reacted with hydroxyl-terminated curing agents during the chain-extending step, as described above, the resulting polyurethane composition contains urethane linkages. On the other hand, when the polyurethane prepolymer is reacted with amine-terminated curing agents during the chain-extending step, any excess isocyanate groups in the prepolymer will react with the amine groups in the curing agent. The resulting polyurethane composition contains urethane and urea linkages and may be referred to as a polyurethane/urea hybrid. The concentration of urethane and urea linkages in the

hybrid composition may vary. In general, the hybrid composition may contain a mixture of about 10 to 90% urethane and about 90 to 10% urea linkages.

More particularly, when the polyurethane prepolymer is reacted with hydroxyl-terminated curing agents during the chain-extending step, as described above, the resulting composition is essentially a pure polyurethane composition containing urethane linkages having the following general structure:



where x is the chain length, i.e., about 1 or greater, and R and R<sub>1</sub> are straight chain or branched hydrocarbon chain having about 1 to about 20 carbons.

However, when the polyurethane prepolymer is reacted with an amine-terminated curing agent during the chain-extending step, any excess isocyanate groups in the prepolymer will react with the amine groups in the curing agent and create urea linkages having the following general structure:



where x is the chain length, i.e., about 1 or greater, and R and R<sub>1</sub> are straight chain or branched hydrocarbon chain having about 1 to about 20 carbons.

The polyurethane compositions used to form the cover layer may contain other polymer materials including, for example: aliphatic or aromatic polyurethanes, aliphatic or aromatic polyureas, aliphatic or aromatic polyurethane/urea hybrids, olefin-based copolymer ionomer compositions, polyethylene, including, for example, low density polyethylene, linear low density polyethylene, and high density polyethylene; polypropylene; rubber-toughened olefin polymers; acid copolymers, for example, poly(meth)acrylic acid, which do not become part of an ionomeric copolymer; plastoelomers; flexomers; styrene/butadiene/styrene block copolymers; styrene/ethylene-butylene/styrene block copolymers; dynamically vulcanized elastomers; copolymers of ethylene and vinyl acetates; copolymers of ethylene and methyl acrylates; polyvinyl chloride resins; polyamides, poly(amide-ester) elastomers, and graft copolymers of ionomer and polyamide including, for example, Pebax<sup>®</sup> thermoplastic polyether block amides, available from Arkema Inc; cross-linked trans-polyisoprene and blends thereof; polyester-based thermoplastic elastomers, such as Hytrel<sup>®</sup>, available from DuPont; polyurethane-based thermoplastic elastomers, such as Elastollan<sup>®</sup>, available from BASF; polycarbonate/polyester blends such as Xylex<sup>®</sup>, available from SABIC Innovative Plastics; maleic anhydride-grafted polymers such as Fusabond<sup>®</sup>, available from DuPont; and mixtures of the foregoing materials.

In addition, the polyurethane compositions may contain fillers, additives, and other ingredients that do not detract from the properties of the final composition. These additional materials include, but are not limited to, catalysts, wetting agents, coloring agents, optical brighteners, cross-linking agents, whitening agents such as titanium dioxide and zinc oxide, ultraviolet (UV) light absorbers, hindered amine light stabilizers, fluorosurfactants, defoaming agents, processing aids, surfactants, and other conventional additives. Other suitable additives include antioxidants, stabilizers, softening agents, plasticizers, including internal and external plasticizers, impact modifiers, foaming agents, density-adjusting fillers, reinforcing materials, compatibilizers, and the like. Some examples of useful fillers include zinc oxide, zinc sulfate, barium carbonate, barium sulfate, calcium oxide, calcium carbonate, clay, tungsten, tungsten carbide, silica, and mixtures thereof. Rubber regrind (recycled core material) and polymeric, ceramic, metal, and glass microspheres also may be used. Generally, the additives will be present in the composition in an amount between about 1 and about 70 weight percent based on total weight of the composition depending upon the desired properties. These additives may be optionally included in the topcoat formulation of this invention as described further below.

#### Intermediate Layers

In one preferred embodiment, an intermediate layer is disposed between the single or multi-layered core and surrounding cover layer. These intermediate layers also can be referred to as casing or mantle or inner cover layers. The intermediate layer can be formed from any materials known in the art, including thermoplastic and thermosetting materials, but preferably is formed of an ionomer composition comprising an ethylene acid copolymer containing acid groups that are at least partially neutralized. Suitable ethylene acid copolymers that may be used to form the intermediate layers are generally referred to as copolymers of ethylene;  $C_3$  to  $C_8$   $\alpha$ ,  $\beta$ -ethylenically unsaturated mono- or dicarboxylic acid; and optional softening monomer. These ethylene acid copolymer ionomers also can be used to form the inner core and outer core layers as described above. In other embodiments, these thermoplastic ionomer compositions can be used to make the golf ball cover.

Suitable ionomer compositions include partially-neutralized ionomers and highly-neutralized ionomers (HNPs), including ionomers formed from blends of two or more partially-neutralized ionomers, blends of two or more highly-neutralized ionomers, and blends of one or more partially-neutralized ionomers with one or more highly-neutralized ionomers. For purposes of the present disclosure, "HNP" refers to an acid copolymer after at least 70% of all acid groups present in the composition are neutralized. Preferred ionomers are salts of O/X- and O/X/Y-type acid copolymers, wherein O is an  $\alpha$ -olefin, X is a  $C_3$ - $C_8$   $\alpha$ ,  $\beta$ -ethylenically unsaturated carboxylic acid, and Y is a softening monomer. O is preferably selected from ethylene and propylene. X is preferably selected from methacrylic acid, acrylic acid, ethacrylic acid, crotonic acid, and itaconic acid. Methacrylic acid and acrylic acid are particularly preferred. Y is preferably selected from (meth) acrylate and alkyl (meth) acrylates wherein the alkyl groups have from 1 to 8 carbon atoms, including, but not limited to, n-butyl (meth) acrylate, isobutyl (meth) acrylate, methyl (meth) acrylate, and ethyl (meth) acrylate.

Preferred O/X and O/X/Y-type copolymers include, without limitation, ethylene acid copolymers, such as ethylene/(meth)acrylic acid, ethylene/(meth)acrylic acid/maleic

anhydride, ethylene/(meth)acrylic acid/maleic acid mono-ester, ethylene/maleic acid, ethylene/maleic acid mono-ester, ethylene/(meth)acrylic acid/n-butyl (meth)acrylate, ethylene/(meth)acrylic acid/iso-butyl (meth)acrylate, ethylene/(meth)acrylic acid/methyl (meth)acrylate, ethylene/(meth)acrylic acid/ethyl (meth)acrylate terpolymers, and the like. The term, "copolymer," as used herein, includes polymers having two types of monomers, those having three types of monomers, and those having more than three types of monomers. Preferred  $\alpha$ ,  $\beta$ -ethylenically unsaturated mono- or dicarboxylic acids are (meth) acrylic acid, ethacrylic acid, maleic acid, crotonic acid, fumaric acid, itaconic acid. (Meth) acrylic acid is most preferred. As used herein, "(meth) acrylic acid" means methacrylic acid and/or acrylic acid. Likewise, "(meth) acrylate" means methacrylate and/or acrylate.

In a particularly preferred version, highly neutralized E/X- and E/X/Y-type acid copolymers, wherein E is ethylene, X is a  $C_3$ - $C_8$   $\alpha$ ,  $\beta$ -ethylenically unsaturated carboxylic acid, and Y is a softening monomer are used. X is preferably selected from methacrylic acid, acrylic acid, ethacrylic acid, crotonic acid, and itaconic acid. Methacrylic acid and acrylic acid are particularly preferred. Y is preferably an acrylate selected from alkyl acrylates and aryl acrylates and preferably selected from (meth) acrylate and alkyl (meth) acrylates wherein the alkyl groups have from 1 to 8 carbon atoms, including, but not limited to, n-butyl (meth) acrylate, isobutyl (meth) acrylate, methyl (meth) acrylate, and ethyl (meth) acrylate. Preferred E/X/Y-type copolymers are those wherein X is (meth) acrylic acid and/or Y is selected from (meth) acrylate, n-butyl (meth) acrylate, isobutyl (meth) acrylate, methyl (meth) acrylate, and ethyl (meth) acrylate. More preferred E/X/Y-type copolymers are ethylene/(meth) acrylic acid/n-butyl acrylate, ethylene/(meth) acrylic acid/methyl acrylate, and ethylene/(meth) acrylic acid/ethyl acrylate.

The amount of ethylene in the acid copolymer is typically at least 15 wt. %, preferably at least 25 wt. %, more preferably least 40 wt. %, and even more preferably at least 60 wt. %, based on total weight of the copolymer. The amount of  $C_3$  to  $C_8$   $\alpha$ ,  $\beta$ -ethylenically unsaturated mono- or dicarboxylic acid in the acid copolymer is typically from 1 wt. % to 35 wt. %, preferably from 5 wt. % to 30 wt. %, more preferably from 5 wt. % to 25 wt. %, and even more preferably from 10 wt. % to 20 wt. %, based on total weight of the copolymer. The amount of optional softening comonomer in the acid copolymer is typically from 0 wt. % to 50 wt. %, preferably from 5 wt. % to 40 wt. %, more preferably from 10 wt. % to 35 wt. %, and even more preferably from 20 wt. % to 30 wt. %, based on total weight of the copolymer. "Low acid" and "high acid" ionomeric polymers, as well as blends of such ionomers, may be used. In general, low acid ionomers are considered to be those containing 16 wt. % or less of acid moieties, whereas high acid ionomers are considered to be those containing greater than 16 wt. % of acid moieties.

The various O/X, E/X, O/X/Y, and E/X/Y-type copolymers are at least partially neutralized with a cation source, optionally in the presence of a high molecular weight organic acid, such as those disclosed in U.S. Pat. No. 6,756,436, the entire disclosure of which is hereby incorporated herein by reference. The acid copolymer can be reacted with the optional high molecular weight organic acid and the cation source simultaneously, or prior to the addition of the cation source. Suitable cation sources include, but are not limited to, metal ion sources, such as compounds of alkali metals, alkaline earth metals, transition metals, and

rare earth elements; ammonium salts and monoamine salts; and combinations thereof. Preferred cation sources are compounds of magnesium, sodium, potassium, cesium, calcium, barium, manganese, copper, zinc, lead, tin, aluminum, nickel, chromium, lithium, and rare earth metals.

Other suitable thermoplastic polymers that may be used to form the intermediate layer include, but are not limited to, the following polymers (including homopolymers, copolymers, and derivatives thereof): (a) polyester, particularly those modified with a compatibilizing group such as sulfonate or phosphonate, including modified poly(ethylene terephthalate), modified poly(butylene terephthalate), modified poly(propylene terephthalate), modified poly(trimethylene terephthalate), modified poly(ethylene naphthalene), and those disclosed in U.S. Pat. Nos. 6,353,050, 6,274,298, and 6,001,930, the entire disclosures of which are hereby incorporated herein by reference, and blends of two or more thereof; (b) polyamides, polyamide-ethers, and polyamide-esters, and those disclosed in U.S. Pat. Nos. 6,187,864, 6,001,930, and 5,981,654, the entire disclosures of which are hereby incorporated herein by reference, and blends of two or more thereof; (c) polyurethanes, polyureas, polyurethane-polyurea hybrids, and blends of two or more thereof; (d) fluoropolymers, such as those disclosed in U.S. Pat. Nos. 5,691,066, 6,747,110 and 7,009,002, the entire disclosures of which are hereby incorporated herein by reference, and blends of two or more thereof; (e) polystyrenes, such as poly(styrene-co-maleic anhydride), acrylonitrile-butadiene-styrene, poly(styrene sulfonate), polyethylene styrene, and blends of two or more thereof; (f) polyvinyl chlorides and grafted polyvinyl chlorides, and blends of two or more thereof; (g) polycarbonates, blends of polycarbonate/acrylonitrile-butadiene-styrene, blends of polycarbonate/polyurethane, blends of polycarbonate/polyester, and blends of two or more thereof; (h) polyethers, such as polyarylene ethers, polyphenylene oxides, block copolymers of alkenyl aromatics with vinyl aromatics and polyamicesters, and blends of two or more thereof; (i) polyimides, polyetherketones, polyamideimides, and blends of two or more thereof; and (j) polycarbonate/polyester copolymers and blends.

#### Golf Ball Construction

The solid cores for the golf balls of this invention may be made using any suitable conventional technique such as, for example, compression or injection-molding. Typically, the cores are formed by compression molding a slug of uncured or lightly cured rubber material into a spherical structure. Prior to forming the cover layer, the core structure may be surface-treated to increase the adhesion between its outer surface and adjacent layer. Such surface-treatment may include mechanically or chemically-abrading the outer surface of the core. For example, the core may be subjected to corona-discharge, plasma-treatment, silane-dipping, or other treatment methods known to those in the art.

Retractable pin injection-molding (RPIM) methods generally involve using upper and lower mold cavities that are mated together. The upper and lower mold cavities form a spherical interior cavity when they are joined together. The mold cavities used to form the outer cover layer have interior dimple cavity details. The cover material conforms to the interior geometry of the mold cavities to form a dimple pattern on the surface of the ball. The injection-mold includes retractable support pins positioned throughout the mold cavities. The retractable support pins move in and out of the cavity. The support pins help maintain the position of the core or ball sub-assembly while the molten composition flows through the mold gates. The molten composition flows into the cavity between the core and mold cavities to

surround the core and form the cover layer. Other methods can be used to make the cover including, for example, reaction injection-molding (RIM), liquid injection-molding, casting, spraying, powder-coating, vacuum-forming, flow-coating, dipping, spin-coating, and the like.

As discussed above, an inner cover layer or intermediate layer, preferably formed from an ethylene acid copolymer ionomer composition, can be formed between the core or ball sub-assembly and cover layer. The intermediate layer comprising the ionomer composition may be formed using a conventional technique such as, for example, compression or injection-molding. For example, the ionomer composition may be injection-molded or placed in a compression mold to produce half-shells. These shells are placed around the core in a compression mold, and the shells fuse together to form an intermediate layer. Alternatively, the ionomer composition is injection-molded directly onto the core using retractable pin injection-molding.

#### Application of Primer, Top-Coats and Isocyanate Treatments

After the golf balls have been removed from the mold, they may be subjected to finishing steps including flash-trimming, surface-treatment, marking, and application of coatings in accordance with this invention. For example, the outer cover layer may be surface-treated using any suitable method such as, for example, corona, plasma, or ultraviolet (UV) light-treatment.

The balls of this invention may be produced in a wide variety of colors, such as white, yellow, orange, green, red, and pink, and are typically colored by painting the outer surface of the ball, or by incorporating pigment directly into the cover composition as discussed above. Normally, the ball also is printed with some type of indicia such as a trademark, tradename, logo, symbol, letter, number, or the like.

For the mass-production of balls, a standard identifying mark is printed on the ball, and the ink can be applied directly onto the cover or a primer coat. For example, a colored or transparent primer paint can be applied first to the surface of the ball and then ink can be applied over the primer to form the indicia, and then a clear top-coat layer can be applied over the indicia. This transparent topcoat layer protects the printed indicia, provides high gloss, provide abrasion or wear-resistance, and generally enhances the overall aesthetics of the ball. Different printing techniques may be used including, for example, using pad-printing, ink-jet printing, dye-sublimation, and the like. The primer and topcoats can be clear or colored. For custom balls that are marked with a custom logo, the ink is often applied to the topcoat of the finished balls. Therefore, an ink that cures rapidly to prevent the smearing and transfer of the ink to other custom balls or to ball printing and handling equipment is required.

Different chemical agents are commonly used in the golf ball components to protect the ball from the harmful effects of ultraviolet (UV) from sunlight and other sources. In general, UV radiation has wavelengths in the range between about 300 to about 400 nm and makes up about 4 to 7% of the total solar radiation. When a golf ball component, for example, a cover material or coating overlying the cover, are exposed to UV radiation, this initiates degradation a photo-oxidative process. The UV radiation from sunlight and other sources can cause discoloration, changes in gloss, and chalking.

The topcoat normally contains light stabilizers and optical brighteners, which both compete for absorption of the ultraviolet (UV) light. Optical brighteners absorb electromag-

netic radiation in the ultraviolet portion of the spectrum and re-emit (ie., "fluoresce") radiation in the visible portion of the spectrum. When applied to the exterior of a golf ball, optical brighteners enhance the whiteness and/or brightness of such balls. This whitening effect makes the materials appear less yellowish by increasing the overall amount of blue light reflected. In general, the brighteners are selected from one of the following classes: triazine-stilbenes (di, tetra-, or hexa-sulfonated); coumarins; imidazolines; diazoles; triazoles; benzoxazolines; and biphenyl-stilbenes; and mixtures thereof.

However, because the molecular structure of optical brighteners typically includes aromatic moieties, optical brighteners can contribute to the discoloration of the top-coat. When exposed to high intensity sunlight, the optical brighteners absorb the ultraviolet (UV) light. In turn, the aromatic or other moieties in the optical brighteners may produce free radicals or there may be a rearrangement of electrons. This results in the production of chromophores that cause the topcoat to visibly discolor if the chromophores are present in a high quantity. For example, the topcoat can develop a yellowish-greenish discoloration in some instances when the concentration of optical brighteners is too great and there is prolonged exposure to sunlight. The absorption of UV light by the high concentration of optical brighteners which are used to obtain the desired brightness may produce a large number of chromophores, and this may cause discoloration such as a greening effect on the ball's cover surface.

Light stabilizers protect against photodegradation initiated due to exposure to UV light. When the coating is exposed to UV radiation from the sunlight, this initiates degradation through a photo-oxidative process. Photo-oxidation is a chain-reaction process involving free radicals and hydroperoxide intermediates. Light stabilizers inhibit this process by absorption of the damaging UV radiation or by scavenging the reactive intermediates. Such stabilizers include ultraviolet (UV) absorbers which absorb ultraviolet radiation and have a high degree of inherent photostability; and hindered amine light stabilizers (HALs) which primarily function by scavenging the free-radical intermediates in the photo-oxidation process. These scavengers interrupt free radical reactions.

Suitable UV absorbers include, but are not limited to, triazines, benzoxazinones, benzotriazoles, benzophenones, benzoates, and the like. In some instances, light stabilizers such as Tinuvin®571, 123, P, and 328, and 329 UV absorbers, commercially available from BASF, are included in the cover material. Adding the light stabilizers to the cover composition can help slow down discoloration due to exposure to the UV radiation. For example, the light stabilizers can be present in the cover composition in an amount in the range of about 1 to about 8 weight percent (wt. %) based on the weight of the composition. In other instances, the cover stock does not include any light stabilizers.

Preferably, the topcoat composition used for coating golf balls of this invention is a polyurethane, solvent-borne composition comprising a resin component and an isocyanate component. The Part A component of the coating preferably contains polyol, catalyst, solvent, UV absorbers, hindered amine light stabilizers, and optical brighteners as described further below. The Part B component of this coating preferably contains polyisocyanates such as hexamethylene diisocyanate, trimer of hexamethylene diisocyanate, or biuret of hexamethylene diisocyanate and solvents as also described further below. Aliphatic isocyanates are preferred since they have better ultraviolet (UV) light dura-

bility and lesser tendency to yellow when exposed to heat and light. The viscosity of the coating is adjusted using solvents including n-butyl acetate, t-butyl acetate, methyl amyl ketone (MAK), and ethyl acetate. Optionally the coating may contain inorganic pigments/fillers such as titanium dioxide, silica, inorganic clay, calcium carbonate, aluminum oxide, and the like. Other solvent-borne formulations such as polyureas, acrylic polyurethanes, polyesters, polyester acrylics, and epoxies also can be used in accordance with this invention.

## EXAMPLES

The invention is further illustrated by the following examples, but these examples should be construed as limiting the scope of the invention. In the following Examples, golf balls comprising a rubber core having a diameter of about 1.550"; a casing formed from an ethylene acid copolymer ionomer composition, wherein the cased core has an outer diameter of about 1.61 inches; and a thermoplastic polyurethane cover were coated with a primer coat and dried. Then, the golf ball samples were top-coated with a clear formulation prepared by mixing Part A with Part B as described below.

The Part A component preferably comprises the following ingredients: polyol (about 30 to about 60 wt. %); catalyst (about 0.1 to about 5.0 wt. %); solvent (about 40 to about 70 wt. %); fluorosurfactant (about 0.1 to about 3.0 wt. %); UV absorbers (about 0.1 to about 5.0 wt. %); hindered amine light stabilizers (about 0.1 to about 5.0 wt. %); and optical brighteners (about 0.01 to about 3.00 wt. %).

In the present invention, it has been found that the topcoat formulation may contain a relatively small amount of optical brightener and this concentration of optical brightener is sufficient to provide good durability, high brightness, prevent discoloration, and enhance the overall aesthetics of the ball. The golf balls of this invention are aesthetically pleasing and have high brightness and good color stability. These golf balls also have high impact durability, namely improved cut and scuff (groove shear) resistance. In a preferred embodiment, the concentration of optical brightener in the topcoat composition is in the range of about 0.01 to about 3.00 wt. %. In another preferred embodiment, the concentration of optical brightener is in the range of about 0.01 to about 0.20 wt. %, more preferably in the range of about 0.1 to about 1.0 wt. %, and even more preferably in the range of about 0.1 to about 0.5 wt. %. In a particularly preferred embodiment, the concentration of optical brightener is in the range of about 0.01 to about 0.2 wt. %. The topcoat of this invention has high uniformity and is durable. The top coating of this invention has substantially uniform thickness. There is high uniform coverage of the top coating over the ball. This coating uniformity is important, because it affects the lift, drag, and flight stability of the ball when the ball is struck with the golf club face. Preferably, the wet weight of the top coat is in the range of about 0.20 g to about 0.42 g based on 3 ball wet weight after one minute in ambient temperature.

The Part B component preferably comprises the following ingredients: polyisocyanate (about 10 to about 100 wt. %) and solvent (about 0 to about 90 wt. %). Suitable polyisocyanates polyols, catalysts, solvents, and fillers are described further below.

In the following Example 1, a topcoat comprising the formulation as described above and containing 0 wt. % Tinuvin and 0 wt. % other light stabilizers and 1 to 3 wt. %

optical brightener was used to coat the TPU cover. The results are shown below in Table 1.

TABLE 1

| SAMPLE      | L*    | A*    | B*    | C*    | H°     | DL*   | DA*   | DB*   | DECMC |
|-------------|-------|-------|-------|-------|--------|-------|-------|-------|-------|
| F (5 hrs.)  | 90.20 | -5.68 | -0.44 | 5.70  | 184.48 | -0.44 | -2.80 | 7.24  | 9.44  |
| G (10 hrs.) | 89.42 | -7.35 | 4.62  | 8.68  | 147.88 | -1.22 | -4.47 | 12.30 | 16.34 |
| H (20 hrs.) | 89.88 | -9.09 | 9.95  | 13.48 | 132.43 | -0.76 | -6.21 | 17.63 | 22.89 |
| I (40 hrs.) | 89.83 | -9.23 | 11.97 | 15.12 | 127.65 | -0.81 | -6.35 | 19.65 | 25.09 |
| J (80 hrs.) | 88.96 | -8.04 | 10.82 | 13.48 | 126.61 | -1.68 | -5.15 | 18.50 | 23.55 |

DECMC—L\* a\* b\* C\* and h° values were measured in the CIELAB color space for each of these constructions using a MacBeth Color-Eye® 7000A spectrophotometer before and after QUV exposure. DECMC (Total Color Difference) is calculated based on delta L\*, a\* b\* color differences using standard techniques. The golf balls were exposed to UV radiation by placing the balls under a Xenon lamp for different time periods (5, 10, 20, 40, or 80 hours.)

Thus, the golf balls shown in Table 1 has a relatively high concentration of optical brightener which is normally used in the topcoat to provide the desired brightness when

exposed to UV radiation by placing the balls under a Xenon lamp for different time periods (5, 10, 20, 40, or 80 hours.)

In the following Example 3, a topcoat comprising the formulation as described above and containing 0 wt. % Tinuvin and 0 wt. % other light stabilizers used to coat the TPU cover. The average three ball wet weight of the coating after drying for one minute at ambient temperature was high weight (greater than 0.40 grams and preferably in the range of about 0.41 to about 0.42 grams). The results are shown below in Table 3.

TABLE 3

| SAMPLE      | L*    | A*    | B*    | C*   | H°     | DL*   | DA*   | DB*   | DECMC |
|-------------|-------|-------|-------|------|--------|-------|-------|-------|-------|
| P (5 hrs.)  | 90.06 | -5.40 | -0.36 | 5.42 | 183.80 | -0.04 | -1.71 | 4.47  | 5.88  |
| Q (10 hrs.) | 89.52 | -6.31 | 2.88  | 6.93 | 155.48 | -0.57 | -2.61 | 7.71  | 10.02 |
| R (20 hrs.) | 89.35 | -7.06 | 5.43  | 8.90 | 142.42 | -0.74 | -3.36 | 10.26 | 13.16 |
| S (40 hrs.) | 89.48 | -6.92 | 5.53  | 8.85 | 141.37 | -0.61 | -3.22 | 10.36 | 13.22 |
| T (80 hrs.) | 89.85 | -6.95 | 6.25  | 9.35 | 138.01 | -0.24 | -3.25 | 11.09 | 14.04 |

exposed to sunlight. However, this high concentration of optical brightener can lead to discoloration problems. Particularly, the balls may develop a yellowish-greenish tint. This greening effect alters the surface of the ball and makes the balls have an unpleasing appearance. For example, each of the golf balls had a golf ball color stability difference (DECMC) of greater than 9.00 when exposed to UV radiation for 5 hours, and greater than 23.00 when exposed to UV radiation for 80 hours.

In the following Example 2, a topcoat comprising the formulation as described above and containing 0 wt. % Tinuvin and 0 wt. % other light stabilizers; and 0.01 to 0.5 wt. % optical brightener was used to coat the TPU cover. The average three ball wet weight of the coating after drying for one minute at ambient temperature was low weight (i.e., in the range of about 0.20 to about 0.40 grams). The results are shown below in Table 2.

DECMC—L\* a\* b\* C\* and h° values were measured in the CIELAB color space for each of these constructions using a MacBeth Color-Eye® 7000A spectrophotometer before and after QUV exposure. DECMC (Total Color Difference) is calculated based on delta L\*, a\* b\* color differences using standard techniques. The golf balls were exposed to UV radiation by placing the balls under a Xenon lamp for different time periods (5, 10, 20, 40, or 80 hours.)

The topcoat of this invention includes a relatively small amount of optical brightener. Preferably, it is in the range of about 0.01 to 0.5% and more preferably 0.01 to 0.2%. The final level of optical brightener is reduced by an amount of at least 5%, preferably 10%, and even more preferably at least 20% over standard top coat formulations containing optical brightener. it has been found that the topcoat formulation may contain a relatively small amount of optical brightener and this concentration of optical brightener is

TABLE 2

| SAMPLE      | L*    | A*    | B*   | C*   | H°     | DL*   | DA*   | DB*   | DECMC |
|-------------|-------|-------|------|------|--------|-------|-------|-------|-------|
| K (5 hrs.)  | 90.16 | -5.59 | 0.47 | 5.61 | 175.16 | -0.20 | -1.86 | 5.00  | 6.56  |
| L (10 hrs.) | 89.79 | -6.59 | 3.30 | 7.37 | 153.38 | -0.57 | -2.87 | 7.83  | 10.21 |
| M (20 hrs.) | 89.90 | -6.89 | 4.04 | 7.99 | 149.60 | -0.46 | -3.17 | 8.57  | 11.15 |
| N (40 hrs.) | 89.88 | -6.88 | 5.28 | 8.67 | 142.50 | -0.48 | -3.15 | 9.80  | 12.52 |
| O (80 hrs.) | 89.61 | -6.68 | 6.01 | 8.99 | 138.02 | -0.75 | -2.96 | 10.54 | 13.30 |

DECMC—L\* a\* b\* C\* and h° values were measured in the CIELAB color space for each of these constructions using a MacBeth Color-Eye® 7000A spectrophotometer before and after QUV exposure. DECMC (Total Color Difference) is calculated based on delta L\*, a\* b\* color differences using standard techniques. The golf balls were

sufficient to provide good durability, high brightness, prevent discoloration, and enhance the overall aesthetics of the ball as shown in the above Tables 3 and 4. For example, each of the golf balls had a golf ball color stability difference (DECMC) of less than 7.00 when exposed to UV radiation for 5 hours; and less than 15.00 when exposed to UV

radiation for 80 hours. The topcoat composition of this invention has a sufficient amount of optical brighteners to provide the desired brightness to the golf ball; and yet at the same time, the ball does not suffer from discoloration problems such as a greening effect when exposed to sunlight. Furthermore, the topcoat of this invention has good uniformity and impact durability.

In another embodiment, a first (primer) polyurethane coating comprising unreacted isocyanate groups and having an isocyanate index of at least about 115 is applied to the outer cover. The golf ball is then preferably treated with heat so the coating is at least partially-cured. For example, the golf ball can be heated preferably to a surface temperature of at least about 1050 to about 200° F. Preferably, the golf ball is heated to a surface temperature of about 120 to about 150° F. Preferably, the golf ball is then heated for at a period of 2 minutes to about 240 minutes, more preferably a period of 4 minutes to 120 minutes, and most preferably about 8 minutes to 60 minutes. In a third step, a second (top-coat) polyurethane coating is applied to the outer cover. Any suitable coating technique may be used to apply the first and second polyurethane coatings. For example, spraying, dipping, brushing, or rolling methods can be used. Then the golf ball can go through a series of finishing steps.

In a second embodiment, a first (primer) polyurethane comprising unreacted isocyanate groups and having an isocyanate index of at least about 115 is applied to the outer cover and the golf ball is treated with heat as described above. In a third step, a second (top-coat) polyurethane coating having an isocyanate index of less than 96 is applied to the outer cover.

In a third embodiment, a first (primer) polyurethane comprising unreacted isocyanate groups and having an isocyanate index of at least about 115 and further comprising a catalyst is applied to the outer cover and the golf ball is treated with heat as described above. In a third step, a second (top-coat) polyurethane coating is applied to the outer cover as described above. The thermoplastic polyurethane composition of the outer cover layer and second (top-coat) polyurethane coatings also may comprise catalysts. Suitable catalysts include, for example, dibutyl tin dilaurate, dibutyl tin acetylacetone, dibutyl tin dibutoxide, dibutyl tin sulfide, dibutyl tin di-2-ethylhexanoate, dibutyl tin (IV) diacetate, dialkyltin (IV) oxide, tributyl tin laurylmercaptate, dibutyl tin dichloride, organo lead, tetrabutyl titanate, tertiary amines, mercaptides, stannous octoate, potassium octoate, zinc octoate, diaza compounds, and potassium acetate, and mixtures thereof.

In a fourth embodiment, a mixture comprising a multi-functional isocyanate and solvent is applied to the outer cover and the golf ball is treated with heat as described above. The mixture also may contain additives such as, for example, ultraviolet (UV) light stabilizers. A first (primer) polyurethane coating that may be over-indexed or under-indexed may be applied to the outer cover. For example, the mixture may be over-indexed and comprise unreacted isocyanate groups and have an isocyanate index of at least about 115. In another example, the mixture may be under-indexed and have an isocyanate index of less than 96. The golf ball is treated with heat as described above. A second polyurethane top-coating having an isocyanate index that is over-indexed or under-indexed may be applied. This treatment of the outer cover layer with isocyanates further enhances cross-linking and improve cover durability. These isocyanates can function as cross-linkers in the thermoplastic polyurethane cover. The chain length of the thermoplastic

polyurethane is extended and thus the molecular weight of the polyurethane is increased when treated with the multi-functional isocyanates.

Isocyanate Indexing: In some embodiments, the cross-linking may take place as a result of the relative proportions of isocyanate functional groups in the cover layer and the coating layer. As is generally known, polyurethanes (whether thermoplastic or thermoset) are polymerized through the reaction between an isocyanate functional group 10 on a polyisocyanate and a hydroxyl functional group on a polyol. The relative stoichiometric amounts of each of these functional groups is expressed as the "isocyanate index" of 15 the polyurethane system. Namely, the isocyanate index may be expressed as the ratio of the number of isocyanate groups present in the polyurethane system to the number of hydroxyl groups times 100. Or, in other words, the isocyanate index may be expressed as the ratio of the actual number of isocyanate functional groups present in the polyurethane system to the hypothetical number of isocyanate 20 functional groups necessary to fully react with all of the hydroxyl groups present in the polyurethane system.

The isocyanate index may also be referred to as the "NCO index." The location of the decimal place may vary based on common convention (i.e. the value of the isocyanate index 25 may be equally expressed as 1.00 or 100 depending on colloquialism). As used herein, an isocyanate index value of 100 means that the number of isocyanate functional groups present in the polyurethane system is equal to the number of hydroxyl functional groups present in the polyurethane 30 system. An isocyanate index value of less than 100 means that excess hydroxyl groups are present, and an isocyanate index value of greater than 100 means that excess isocyanate groups are present.

Preferably, the multi-functional isocyanate compound is 35 selected from the group consisting of toluene 2,4-diisocyanate (TDI), toluene 2,6-diisocyanate (TDI), 4,4'-methylene diphenyl diisocyanate (MDI), 2,4'-methylene diphenyl diisocyanate (MDI), polymeric methylene diphenyl diisocyanate (PMDI), p-phenylene diisocyanate (PPDI), m-phenylene diisocyanate (PDI), naphthalene 1,5-diisocyanate (NDI), naphthalene 2,4-diisocyanate (NDI), p-xylene diisocyanate (XDI), and isophorone diisocyanate (IPDI), 1,6-hexamethylene diisocyanate (HDI), 4,4'-dicyclohexylmethane diisocyanate ("H<sub>12</sub> MDI"), meta-tetramethylxylylene diisocyanate (TMXDI), trans-cyclohexane diisocyanate (CHDI), and homopolymers and copolymers and blends thereof. More preferably, the polyisocyanate is selected from the group consisting of 4,4'-methylene diphenyl diisocyanate (MDI), 2,4'-methylene diphenyl diisocyanate (MDI), toluene 2,4-diisocyanate (TDI), toluene 2,6-diisocyanate (TDI), 4,4'-dicyclohexylmethane diisocyanate ("H<sub>12</sub> MDI"), p-phenylene diisocyanate (PPDI), and isophorone diisocyanate (IPDI), and homopolymers and copolymers and blends thereof.

Generally, the polyurethane coating material may be a two-part coating system. A preferred coating system includes (1) a first part comprising a polyol or another compound containing an active hydrogen atom, and (2) a second part comprising a polyisocyanate (or polyisocyanurate) with at least two —N=C=O groups. Suitable polyols for the polyurethane coating system include both polyether and polyester polyols. In one particular embodiment, the polyol may be a hydroxyl functional polyol having a hydroxyl equivalent weight in the range of from about 50 to 60 about 1500, or a hydroxyl equivalent weight being in the range of from about 200 to about 800. Suitable polyesters for use herein include poly (oxydiethylene adipates) that are

condensation products of diethylene glycol and adipic acid, branched with trimethylolpropane or pentaerythritol, and polycaprolactone (hydroxycaproic acid) polyesters.

The solvent may be any solvent that forms a solution with the multi-functional isocyanate and allows for some level of penetration of the isocyanate into the thermoplastic polyurethane substrate to which it is applied. Suitable solvents include, for example, toluene, xylene, naphthalene, ketones, and acetates. Preferably, the solvent comprises one selected from the group consisting of acetone, methyl ethyl ketone, methyl amyl ketone, dimethyl heptanone, methyl pentanone, methyl isobutyl ketone, cyclohexanone, methyl acetate, ethyl acetate, and butyl acetate, and mixtures thereof. The mixture preferably comprises from about 1 to 25 wt. % isocyanate, and more preferably about 2 to 20 wt. %, and most preferably 5 to 18 wt % isocyanate.

The polyurethane coating material may also be formed from a polyurethane system that includes a catalyst. Generally, the catalyst increases the rate of curing. The catalyst may comprise at least one member selected from the group consisting of dibutyl tin dilaurate, dibutyl tin acetylacetone, dibutyl tin dibutoxide, dibutyl tin sulphide, dibutyl tin di-2-ethylhexanoate, dibutyl tin (IV) diacetate, dialkyltin (IV) oxide, tributyl tin laurylmercaptide, dibutyl tin dichloride, organo lead, tetrabutyl titanate, tertiary amines, mercaptides, stannous octoate, potassium octoate, zinc octoate, diaza compounds, and potassium acetate.

The catalyst may be present in a quantity of 0.01-10 weight active catalyst (not including any carrier) based on total resin solids (polyol plus polyisocyanate, excluding solvents). The quantity of catalyst will depend upon the type of catalyst, polyol, polyisocyanate, and solvents which are used, as well as the curing temperature and desired curing time. For example, when dibutyl tin dilaurate is used as the catalyst, it preferably is present in an amount of about 0.05-0.35 weight % active catalyst based upon total resin solids, and more preferably 0.08-0.15 weight % based upon total resin solids. Generally, the catalyst preferably is present in an amount sufficient to reduce the curing time of the coating as compared to a coating system which does not contain the catalyst but is otherwise identical.

One embodiment of the invention includes a golf ball comprising a single or dual core and a cover layer formed from a thermoplastic polyurethane (TPU), wherein the TPU cover is not treated with an isocyanate-rich composition as described above. In another embodiment, the TPU cover is treated with an isocyanate-rich composition as described above.

Post-treatment of molded golf balls having thermoplastic polyurethane covers with isocyanate-rich and other compositions are described, for example, in Sullivan and Binette, U.S. Pat. Nos. 10,252,113 and 10,363,458 and published U.S. Patent Applications 2019/0083854-A1 and 2019/0217157-A1, all of the disclosures of which are incorporated by reference.

#### Thickness and Hardness of Golf Balls

The golf balls of this invention provide the ball with a variety of advantageous mechanical and playing performance properties as discussed further below. In general, the hardness, diameter, and thickness of the different ball layers may vary depending upon the desired ball construction. If the ball includes an intermediate layer or inner cover layer, the hardness (material) is about 50 Shore D or greater, more preferably about 55 Shore D or greater, and most preferably about 60 Shore D or greater. In one embodiment, the inner cover has a Shore D hardness of about 62 to about 90 Shore D. In one example, the inner cover has a hardness of about

68 Shore D or greater. In addition, the thickness of the inner cover layer is preferably about 0.015 inches to about 0.100 inches, more preferably about 0.020 inches to about 0.080 inches, and most preferably about 0.030 inches to about 0.050 inches.

The manufacturing methods of this invention may be used to mold relatively thin outer covers, for example covers having a thickness of less than 0.075 inches, more preferably 0.050 inches and below, preferably 0.040 inches and below, 10 more preferably 0.030 inches and below, and most preferably 0.025 inches and below.

More particularly, the outer cover preferably has a thickness within a range having a lower limit of about 0.004 or 15 0.010 or 0.020 or 0.030 or 0.040 inches and an upper limit of about 0.050 or 0.055 or 0.065 or 0.070 or 0.080 inches. Most preferably, the thickness of the outer cover is about 0.025 inches or less. The outer cover preferably has a surface hardness of 65 Shore D or less, or 55 Shore D or less, or 50 Shore D or less, or 50 Shore D or less, or 45 Shore D or less. 20 Preferably, the outer cover has hardness in the range of about 20 to about 59 Shore D. In one example, the outer cover has hardness in the range of about 25 to about 55 Shore D.

The manufacturing method of this invention is particularly effective in providing golf balls having a thin outer cover layer. Furthermore, the method of this invention provides thin outer covers with substantially uniform thickness. The resulting balls of this invention have good impact durability and cut/shear-resistance. The United States Golf Association ("USGA") has set total weight limits for golf balls. Particularly, the USGA has established a maximum weight of 45.93 g (1.62 ounces) for golf balls. There is no lower weight limit. In addition, the USGA requires that golf balls used in competition have a diameter of at least 1.68 inches. There is no upper limit so many golf balls have an 30 overall diameter falling within the range of about 1.68 to about 1.80 inches. The golf ball diameter is preferably about 1.68 to 1.74 inches, more preferably about 1.68 to 1.70 inches. In accordance with the present invention, the weight, diameter, and thickness of the core and cover layers may be 35 adjusted, as needed, so the ball meets USGA specifications of a maximum weight of 1.62 ounces and a minimum diameter of at least 1.68 inches.

Preferably, the golf ball has a Coefficient of Restitution (COR) of at least 0.750 and more preferably at least 0.800 45 (as measured per the test methods below.) The core of the golf ball generally has a compression in the range of about 30 to about 130 and more preferably in the range of about 70 to about 110 (as measured per the test methods below.) These properties allow players to generate greater ball 50 velocity off the tee and achieve greater distance with their drives. At the same time, the relatively thin outer cover layer means that a player will have a more comfortable and natural feeling when striking the ball with a club. The ball is more playable and its flight path can be controlled more easily. 55 This control allows the player to make better approach shots near the green. Furthermore, the outer covers of this invention have good impact durability and mechanical strength.

Referring to FIG. 1, a front view of a finished golf ball that can be made in accordance with this invention is generally indicated at (10). The dimples (12) may have various shapes and be arranged in various patterns to modify the aerodynamic properties of the ball. The dimples (112) may have various shapes and be arranged in various patterns to modify the aerodynamic properties of the ball. As discussed above, 60 the polymeric cover material conforms to the interior geometry of the mold cavities to form a dimple pattern on the surface of the ball. The mold cavities may have any suitable 65

dimple arrangement such as, for example, icosahedral, octahedral, cube-octahedral, dipyrad, and the like. In addition, the dimples may be circular, oval, triangular, square, pentagonal, hexagonal, heptagonal, octagonal, and the like. Possible cross-sectional shapes include, but are not limited to, circular arc, truncated cone, flattened trapezoid, and profiles defined by a parabolic curve, ellipse, semi-spherical curve, saucer-shaped curve, sine or catenary curve, or conical curve. Other possible dimple designs include dimples within dimples, constant depth dimples, or multi-lobe dimples. It also should be understood that more than one shape or type of dimple may be used on a single ball, if desired. The total number of dimples on the ball, or dimple count, may vary depending such factors as the sizes of the dimples and the pattern selected. Dimple patterns that provide a high percentage of surface coverage are preferred.

As shown in FIG. 2, a two-piece golf ball (14) can be made having a core (16) and a surrounding thermoplastic polyurethane outer cover layer (18). In the golf ball (14), the core (16) has a relatively large diameter and the outer cover (18) has a relatively small thickness. Referring to FIG. 3, in another embodiment, a two-piece golf ball (20) having a smaller core (22) and a thicker outer cover layer (24) can be made. Turning to FIG. 4, a three-piece golf ball (26) is made, wherein the dual-layered core (inner core (28) and outer core layer (30)) is surrounded by a single-layered thermoplastic polyurethane cover (32).

In FIG. 5, a partial cut-away view of a three-piece golf ball (42) having an inner core (44), outer core (46) and surrounding thermoplastic polyurethane cover (48) is shown. Finally, in FIG. 6, a four-piece ball (50) containing a dual-core having an inner core (52) and outer core layer (54) is shown. The dual-core is surrounded by a multi-layered cover with an inner cover layer (56) and thermoplastic polyurethane outer cover (60).

It should be understood that the golf balls shown in FIGS. 1-6 are for illustrative purposes only, and they are not meant to be restrictive. Other golf ball constructions can be made in accordance with this invention.

When numerical lower limits and numerical upper limits are set forth herein, it is contemplated that any combination of these values may be used. Other than in the operating examples, or unless otherwise expressly specified, all of the

numerical ranges, amounts, values and percentages such as those for amounts of materials and others in the specification may be read as if prefaced by the word "about" even though the term "about" may not expressly appear with the value, amount or range. Accordingly, unless indicated to the contrary, the numerical parameters set forth in the specification and attached claims are approximations that may vary depending upon the desired properties sought to be obtained by the present invention.

It is understood that the manufacturing methods, compositions, constructions, and products described and illustrated herein represent only some embodiments of the invention. It is appreciated by those skilled in the art that various changes and additions can be made to the methods, compositions, constructions, and products without departing from the spirit and scope of this invention. It is intended that all such embodiments be covered by the appended claims.

We claim:

1. A method for forming a coated golf ball, comprising the steps of:
  - providing a golf ball comprising at least one core layer and an outer cover layer, wherein the outer cover layer is formed from a thermoplastic polyurethane composition;
  - applying a mixture comprising multi-functional isocyanate and solvent to the outer cover layer;
  - applying a first polyurethane coating comprising unreacted isocyanate groups and having an isocyanate index of at least about 115 to the outer cover layer;
  - treating the golf ball with heat; and
  - applying a second polyurethane coating to the outer cover of the golf ball, the second polyurethane coating comprising an optical brightener in a concentration of about 0.01 to about 0.20 weight %, to form a coated golf ball.
2. The method of claim 1, wherein the wet weight of the second polyurethane coating is in the range of about 0.20 g to about 0.42 g.
3. The method of claim 1, wherein the optical brightener is selected from the group consisting of triazine-stilbenes (di-, tetra-, or hexa-sulfonated); coumarins; imidazolines; diazoles; triazoles; benzooxazolines; and biphenyl-stilbenes; and mixtures thereof.

\* \* \* \* \*